

# United States Patent Office

3,110,635

Patented Nov. 12, 1963

1

3,110,635

## NORMALIZED ALLOY STEELS

John A. Gulya, Lancaster, Pa., assignor to Lukens Steel Company, Coatesville, Pa., a corporation of Pennsylvania

No Drawing. Filed July 24, 1961, Ser. No. 128,332  
7 Claims. (Cl. 148—36)

The present invention relates to improved weldable normalized alloy steels characterized by excellent notch toughness throughout a wide range of thicknesses. The present invention further relates to low-carbon low-alloy steels that are particularly useful in structural and pressure vessel applications.

Steels used in structural and pressure vessel applications should exhibit weldability, uniform high strength and notch toughness throughout a wide range of section thicknesses. In order to insure excellent weldability the amount of carbon should be low and the tensile strength and notch toughness of the steel increased with low amounts of selected alloying elements. The problem of selecting the proper balance of alloying elements for a steel useful in structural and pressure vessel applications is a difficult one, especially if substantially uniform properties over a broad range of section thicknesses are to be obtained. This is evidenced in the available steels which exhibit decreased strength accompanied by a marked reduction in notch toughness in the heavier sections.

Efforts to compensate for strength loss by increasing carbon content and quenching from austenizing temperatures result in impairing the weldability, ductility and/or notch toughness characteristics of these steels. Furthermore, most alloy steels, whether of the quenched or normalized types, require a tempering or stress-relieving treatment to develop adequate impact resistance, and many structures or components are of such mass configuration that such treatments are impractical after fabrication. Similarly, increasing the gage is unsatisfactory for economic as well as dimensional reasons.

It is an object of the present invention to provide an improved weldable normalized steel that is characterized by high strength and excellent notch toughness over a broad range of thicknesses.

It is another object of the present invention to provide a low-carbon, low-alloy steel that is particularly useful in structural and pressure vessel applications.

It is still another object of the present invention to provide an economical combination of alloying elements that will have the above desirable characteristics.

These and other objects are achieved with alloys having the following compositions.

Element:

Percent by weight

|            |            |
|------------|------------|
| Carbon     | 0.10—0.28  |
| Manganese  | 0.90—1.40  |
| Phosphorus | Up to 0.04 |
| Sulphur    | Up to 0.05 |
| Silicon    | 0.11—0.40  |
| Nickel     | 0.30—0.80  |

2

|                                                     |                   |
|-----------------------------------------------------|-------------------|
| Element—Continued:                                  | Percent by weight |
| Chromium                                            | 0.50—1.00         |
| Molybdenum                                          | 0.15—0.35         |
| Vanadium                                            | 0.02—0.10         |
| Balance iron and incidental steel-making residuals. |                   |

Preferred alloys are those restricted to the following.

|                                                     |                   |
|-----------------------------------------------------|-------------------|
| Element:                                            | Percent by weight |
| C                                                   | 0.13—0.21         |
| Mn                                                  | 0.95—1.30         |
| P                                                   | Up to 0.035       |
| S                                                   | Up to 0.040       |
| Si                                                  | 0.11—0.30         |
| Ni                                                  | 0.40—0.70         |
| Cr                                                  | 0.60—0.90         |
| Mo                                                  | 0.20—0.30         |
| V                                                   | 0.03—0.08         |
| Balance iron and incidental steel-making residuals. |                   |

The above alloys including the preferred alloys can contain 0.02 to 0.10% aluminum, and other deoxidizers as well as conventional additives used in the preparation of fine-grained steels. Further, the alloys of the present invention can have 0.25—0.45% by weight of copper, replacing a like amount of iron when maximum resistance to atmospheric corrosion is desired.

The following examples are illustrative of the excellent properties of the alloys of the present invention.

### Example I

Sections of approximately six inches of the following alloy were normalized at 1700° F., allowed to cool and tempered at 1100° F. Each heat treatment time was four hours. The alloy analyzed as—

|                                                           |                   |
|-----------------------------------------------------------|-------------------|
| Element:                                                  | Percent by weight |
| C                                                         | 0.16              |
| Mn                                                        | 1.24              |
| P                                                         | 0.020             |
| S                                                         | 0.014             |
| Si                                                        | 0.16              |
| Ni                                                        | 0.60              |
| Cr                                                        | 0.80              |
| Mo                                                        | 0.27              |
| V                                                         | 0.05              |
| Al                                                        | 0.04              |
| Cu                                                        | 0.31              |
| Balance iron and other incidental steel-making residuals. |                   |

After the aforementioned heat treatments, the longitudinal mechanical properties at the quarter line of the plate thickness were determined. Tensile data were obtained from standard 0.505-inch diameter specimens and impact data from standard Charpy V-notch specimens. Results given in the following table show that adequate strength and toughness is provided in heavy sections even without tempering:

|          | Condition                | Yield, p.s.i. | Tensile, p.s.i. | Elongation in 2", Minimum percent | Reduction of Area, percent | Impact at 80° F., ft.-lbs. | Impact at -80° F., ft.-lbs. |
|----------|--------------------------|---------------|-----------------|-----------------------------------|----------------------------|----------------------------|-----------------------------|
| Sample 1 | Normalized.              | 70.4K         | 109.9K          | 21                                | 59.8                       | 59                         | 17                          |
| Sample 2 | Normalized and tempered. | 79.4K         | 101.7K          | 20                                | 60.6                       | 70                         | 22                          |

In order to illustrate the favorable properties of the above steel in lighter gages, a 1" section of the above alloy was normalized at 1700° F. for two hours and stress relieved at 1100° F. for two hours and tested as above. The results of the tests are shown in the following table.

|               | Yield, p.s.i. | Tensile, p.s.i. | E (2'') percent | R.A. | Impact at 80° F., ft.-lbs. | Impact at -80° F., ft.-lbs. | 10 |
|---------------|---------------|-----------------|-----------------|------|----------------------------|-----------------------------|----|
| Sample 3..... | 94.8K         | 116.2K          | 22              | 59.5 | 61                         | 25                          |    |

### Examples II and III

Two additional sections of approximately six inches were normalized at 1700° F. for four hours, air cooled, and tempered at 1100° F. These sections were analyzed as:

| Element | Wt. percent, Example II | Wt. percent, Example III |
|---------|-------------------------|--------------------------|
| C.....  | 0.15                    | 0.17                     |
| Mn..... | 1.28                    | 1.07                     |
| P.....  | 0.008                   |                          |
| S.....  | 0.024                   | 0.025                    |
| Si..... | 0.11                    | 0.14                     |
| Ni..... | 0.58                    | 0.63                     |
| Cr..... | 0.87                    | 1.00                     |
| Mo..... | 0.23                    | 0.27                     |
| V.....  | 0.045                   | 0.048                    |
| Al..... | 0.10                    | 0.02                     |

NOTE.—Balance iron and incidental steel-making residuals for both sections.

Tensile and impact data are recorded in the following table:

|                  | Yield Strength (1,000 p.s.i.) | Tensile Strength (1,000 p.s.i.) | E (2'') | R.A. | Impact at -40° F., ft.-lbs. | Impact at 80° F., ft.-lbs. |
|------------------|-------------------------------|---------------------------------|---------|------|-----------------------------|----------------------------|
| Example II.....  | 89.4                          | 101.7                           | 20      | 60.6 | 24                          |                            |
| Example III..... | 79.0                          | 107.5                           | 21      | 53.9 | 22                          |                            |

The above tests demonstrate that the low alloy steels of the present invention exhibit high strength accompanied by good notch toughness even at low temperatures. These desirable characteristics are present in the heavy sections of the alloy steels in the normalized condition with substantially equally favorable properties in the normalized and stress relieved condition.

The above description and drawings disclose several embodiments of the invention, and specific language has been employed in describing the several figures. It will, nevertheless, be understood that no limitations of the scope of the invention are thereby contemplated, and that various alterations and modifications may be made such as would occur to one skilled in the art to which the invention relates.

I claim:

1. An improved weldable normalized steel consisting essentially of

| Element:                                            | Percent by weight |
|-----------------------------------------------------|-------------------|
| Carbon                                              | 0.10-0.28         |
| Manganese                                           | 0.90-1.40         |
| Phosphorus                                          | Up to 0.04        |
| Sulphur                                             | Up to 0.05        |
| Silicon                                             | 0.11-0.40         |
| Aluminum                                            | 0.02-0.10         |
| Nickel                                              | 0.30-0.80         |
| Chromium                                            | 0.50-1.00         |
| Molybdenum                                          | 0.15-0.35         |
| Vanadium                                            | 0.02-0.10         |
| Balance iron and incidental steel-making residuals, |                   |

said steel being characterized in having high uniform strength and toughness through a wide range of thicknesses.

2. An improved weldable normalized steel consisting essentially of

| Element:                                            | Percent by weight |
|-----------------------------------------------------|-------------------|
| Carbon                                              | 0.13-0.21         |
| Manganese                                           | 0.95-1.30         |
| Phosphorus                                          | Up to 0.035       |
| Sulphur                                             | Up to 0.040       |
| Silicon                                             | 0.11-0.30         |
| Aluminum                                            | 0.02-0.10         |
| Nickel                                              | 0.40-0.70         |
| Chromium                                            | 0.60-0.90         |
| Molybdenum                                          | 0.20-0.30         |
| Vanadium                                            | 0.03-0.08         |
| Balance iron and incidental steel-making residuals, |                   |

20 said steel being characterized in having high uniform strength and toughness through a wide range of thicknesses.

3. An improved weldable normalized steel consisting essentially of

| Element:                                             | Percent by weight |
|------------------------------------------------------|-------------------|
| Carbon                                               | 0.10-0.28         |
| Manganese                                            | 0.90-1.40         |
| Phosphorus                                           | Up to 0.04        |
| Sulphur                                              | Up to 0.05        |
| Silicon                                              | 0.11-0.40         |
| Aluminum                                             | 0.02-0.10         |
| Nickel                                               | 0.30-0.80         |
| Chromium                                             | 0.50-1.00         |
| Molybdenum                                           | 0.15-0.35         |
| Vanadium                                             | 0.02-0.10         |
| Copper                                               | 0.25-0.45         |
| Balance iron and incidental steel-making impurities, |                   |

40 said steel being characterized in having high uniform strength and toughness through a wide range of thicknesses.

4. An improved weldable normalized steel consisting essentially of

| Element:                                             | Percent by weight |
|------------------------------------------------------|-------------------|
| Copper                                               | 0.25-0.45         |
| Carbon                                               | 0.10-0.28         |
| Manganese                                            | 0.90-1.40         |
| Phosphorus                                           | Up to 0.04        |
| Sulphur                                              | Up to 0.05        |
| Silicon                                              | 0.11-0.40         |
| Aluminum                                             | 0.02-0.10         |
| Nickel                                               | 0.30-0.80         |
| Chromium                                             | 0.50-1.00         |
| Molybdenum                                           | 0.15-0.35         |
| Vanadium                                             | 0.02-0.10         |
| Balance iron and incidental steel-making impurities, |                   |

60 said steel being characterized in having high uniform strength and toughness through a wide range of thicknesses.

5. An improved weldable normalized low-alloy steel article consisting essentially of alloying elements of substantially 0.16 percent carbon, 1.24 percent manganese, 0.16 percent silicon, 0.60 percent nickel, 0.80 percent chromium, 0.27 percent molybdenum, 0.05 percent vanadium, 0.04 percent aluminum, 0.31 percent copper, and the remainder iron and impurities and elements in amounts which do not adversely affect the heat treatment characteristics of the steel, and characterized by a tensile strength in excess of 100,000 pounds per square inch through a wide range of thicknesses and high impact resistance in the range of  $\pm 80^\circ$  Fahrenheit.

65

70

75

6. An improved weldable normalized low-alloy steel article consisting essentially of alloying elements of substantially 0.15 percent carbon, 1.28 percent manganese, 0.11 percent silicon, 0.58 percent nickel, 0.87 percent chromium, 0.23 percent molybdenum, 0.045 percent vanadium, 0.10 percent aluminum, and the remainder iron and impurities and elements in amounts which do not adversely affect the heat treatment characteristics of the steel, and characterized by tensile strength in excess of 100,000 pounds per square inch through a wide range of thicknesses and high impact resistance in a range of  $\pm 80^\circ$  Fahrenheit.

7. An improved weldable normalized low-alloy steel article consisting essentially of alloying elements of substantially 0.17 percent carbon, 1.07 percent manganese, 0.14 percent silicon, 0.63 percent nickel, 1.00 percent chromium, 0.27 percent molybdenum, 0.048 percent

vanadium, 0.02 percent aluminum, and the remainder iron and impurities and elements in amounts which do not adversely affect the heat treatment characteristics of the steel, and characterized by a tensile strength in excess of 100,000 pounds per square inch through a wide range of thicknesses and high impact resistance in a range of  $\pm 80^\circ$  Fahrenheit.

## References Cited in the file of this patent

## UNITED STATES PATENTS

|           |                |               |
|-----------|----------------|---------------|
| 1,896,889 | French         | Feb. 7, 1933  |
| 2,140,237 | Leitner        | Dec. 13, 1938 |
| 2,565,953 | Gaspari et al. | Aug. 28, 1951 |

## OTHER REFERENCES

Case et al.: "Al in Iron and Steel," 1953, page 5 relied upon. Published by John Wiley & Sons, New York, N.Y.